# EUROPEAN PATENT SPECIFICATION

(11) **EP 0 046 815 B1**
(45) Date of publication and mention of the grant of the patent: **29.01.1986**
(21) Application number: 80105143.4
(22) Date of filing: 29.08.1980
(51) Int. Cl.: D01D 5/08, D01F 6/62, D01D 5/16

(54) **Continuous spin-draw polyester process**
Verfahren zum kontinuierlichen Spinnstrecken von Polyester
Procédé pour le filage-étirage en continu de polyester

(43) Date of publication of application: 10.03.1982
(73) Proprietor: ALLIED CORPORATION, Morristown New Jersey 07960 (US)
(72) Inventor: Hamlyn, Maxwell Charles, Cary North Carolina 27511 (US)
(74) Representative: Brock, Peter William

## Description

This invention relates to the simultaneous (coupled) spin-drawing of continuous filament synthetic fibers from industrial polyester polymer. More particularly, it relates to an improved process for the production of low shrinkage, continuous polyester fibers which are particularly useful in the preparation of industrial products, including industrial belts, conveyor belts, and reinforced elastomeric structures. Still more particularly, it relates to a continuous process for the production of low shrinkage continuous polyester fibers by melt-spinning the polymer followed immediately by drawing the spun fibers wherein the spun fibers are heated substantially immediately above their second order transition temperature by being passed through a steam impinging draw point localizing jet at a steam temperature of 460°C to 580°C. Yarn thermal shrinkage is reduced and yarn dimensional stability improved with no adverse yarn property changes such as lower strength or higher elongation at break.

### Description of the prior art

There are several prior art processes for reducing thermal shrinkage or polyester yarns; however, this reduction in polyester yarn thermal shrinkage normally can be achieved only by sacrificing strength or mechanical quality, increasing ultimate elongation or elongation at break, or by the expensive alternative of a separate operation following drawing, such as annealing or some other form of heat treatment. It is therefore desirable to have a continuous process which reduces yarn shrinkage without any of the aforementioned disadvantages. In this regard, several processes are known which involve conditions of continuously spinning and drawing filaments. See, for example, U.S. Patent US―A―4 070 432 to Tamaddon.

Other pertinent art is U.S. Patent US―A―4 113 821 to Russell et al. which teaches a process for preparing high strength polyester yarn.

### Summary of the invention

The present invention relates to an improved process for the simultaneous spin-drawing of one or more ends of multifilament, continuous filament, synthetic polyester industrial fiber wherein the improvement comprises localizing the draw point of the fiber through use of a noncondensing steam jet at a stream temperature of about 460°C to 580°C so that a reduced shrinkage industrial fiber is produced.

The present invention also relates to an improved process for the simultaneous spin-drawing of one or more ends of synthetic fibers from an industrial polyester polymer whereby a reduced shrinkage industrial fiber is produced. The process, which includes the steps of supplying a melt of the polymer to a spinning unit, extruding the molten polymer through a spinnerette having a plurality of extrusion orifices into a gaseous medium, cooling the extruded polymer filaments, lubricating the filaments, heating the filaments substantially immediately above their second order transition temperature, drawing and then winding up the filaments, is improved by passing the filaments through a steam impinging draw point localizing jet at a temperature of about 482°C to 580°C to thereby heat the filaments substantially immediately above their second order transition temperature. The percent thermal shrink is reduced without significant effect on other yarn properties.

The present invention further relates to a process for the simultaneous spin-drawing of one or more ends of multifilament, continuous filament, synthetic polyester industrial fiber. This process, in addition to reducing percent thermal shrink, produces a dimensionally stable polyester industrial fiber. The process comprises the steps of:
(a) supplying a melt of polyester polymer to a spinning unit;
(b) extruding the melt through a spinnerette having a plurality of extrusion orifices to form filaments;
(c) advancing the extruded filaments through a substantially stationary column of air contained in a heated sleeve having a temperature of about 200°C. to 350°C.;
(d) advancing the filaments through a quenching zone;
(e) lubricating the filaments;
(f) passing the lubricated filaments over a forwarding roll system maintained at a temperature of less than 50°C.;
(g) subsequently passing the filaments through a steam impinging draw point localizing jet at a steam temperature of about 482°C. to 580°C. to heat the filaments substantially immediately above their second order transition temperature;
(h) passing the filaments over a pair of draw rolls wherein at least one of the draw rolls is maintained at a temperature of between about 190°C. and 237°C.;
(i) passing the filaments over a relax roll system maintained at a temperature of about 60°C. to 135°C., yarn tension to the relax roll system being maintained at about 0.4 to 2.0 grams per denier; and
(j) winding up the filaments at a tension of from about 0.06 to 0.6 gram per denier.

It is preferred that the melt have an intrinsic viscosity of about 0.68 to 0.96, most preferably of about 0.68 to 0.78 and that it be supplied at a temperature of about 272°C. to 310°C. It is also preferred that the steam temperature for localizing the draw point of the fiber be about 510°C. to 580°C.

Throughout the present specification and claims, the intrinsic viscosity of the polyester melt is given as a measure for the mean molecular weight, which is determined by standard procedures wherein the concentration of the measuring solution amounts to 0.5 g./100 mL, the solvent is a 60 percent phenol/40 percent tetrachloroethane mixture, and the measuring temperature is 25°C.

The tenacity or breaking strength in grams per denier (UTS) is defined by ASTM Standards, Part 24, American Society for Testing and Materials, 1916 Race Street, Philadelphia, Pennsylvania, page 33 (1965), as "the maximum resultant internal force that resists rupture in a tension test," or "breaking load or force, expressed in units of weight required to break or rupture a specimen in a tensile test made according to specified standard procedures." By "% U.E." is meant elongation at break in percent.

The term shrinkage is defined as "percent decrease in length of a material when exposed to elevated temperatures for a specified period of time and under 0.05 g.p.d. tension." In the present invention the percent thermal shrinkage (% T.S.) is measured between two metal plates maintained at 177°C. for a time period of 60 seconds.

The term "modulus" in grams per denier, also known as tensile modulus (Young's Modulus), is expressed as the ratio of change in stress to change in strain in the initial straight-line portion of the stress-strain curve extrapolated to 100 percent elongation.

The term "toughness", also known as toughness index, is defined (above reference) as "the actual work per unit volume (or per unit mass) of material which is required to rupture the material. It is proportional to the area under the load-elongation curve from the origin to the breaking point." The toughness index is routinely measured in grams centimeter per denier centimeter.

In measuring yarn quality, the mechanical quality rating is made by visual examination of a stationary package wherein a rating of 1 to 3 to assigned with 1 being excellent and 3 being substandard. A strobe examination is made by flashing a strobe on a rotating package wherein the strobe frequency is identical to the RPMs of the package and wherein a visual rating of 1 to 4 is assigned with 1 being excellent and 4 being unacceptable.

The preferred polyesters are the linear terephthalate polyesters, i.e., polyesters of a glycol containing from 2 to 20 carbon atoms and a dicarboxylic acid component containing at least about 75 percent terephthalic acid. The remainder, if any, of the dicarboxylic acid component may be any suitable dicarboxylic acid such as sebacic acid, adipic acid, isophthalic acid, sulfonyl-4,4'-dibenzoic acid, or 2,8-di-benzofuran-dicarboxylic acid. The glycols may contain more than two carbons atoms in the chain, e.g., diethylene glycol, butylene glycol, decamethylene glycol, and bis - (1,4 - (hydroxymethyl) - cyclohexane. Examples of linear terephthalate polyesters which may be employed include (poly(ethylene terephthalate), poly(ethylene terephthalate/5 - chloroisophthalate) (85/15), poly(ethylene terephthalate/5 - [sodium sulfo] - isophthalate) (97/3), poly(cyclohexane - 1,4 - dimethylene terephthalate), and poly(cyclohexane - 1,4 - dimethylene terephthalate/hexahydroterephthalate) (75/25).

### Brief description of the drawings

Figure is a schematic front view of the apparatus used for the method of this invention, and Figure 2 is a schematic of the draw panel designated by the numeral 21 in Figure 1.

### Description of the preferred embodiment

It has now been found that reduced shrinkage industrial fiber can be melt-spun continuously from a polyester polymer, e.g., polyethylene terephthalate, and that this fiber can be continuously drawn without the intermediate step of winding up. These results are achieved in accordance with this invention by increasing the steam drawing temperature to enhance crystalline development, thereby enabling economic one-step (coupled) production of fibers with improved dimensional stability (the sum of % U.E.+%T.S.) and higher strength (U.T.S.). By "one-step production" is meant that there is no winding up step between the melt spinning and drawing steps, and there is no need for a separate operation or step such as annealing, carried out subsequent to the simultaneous spin-drawing process.

Referring to Figures 1 and 2, like numbers indicate like apparatus. Molten polymer is fed by extruder 11 to spin pump 12 which feeds spin block 13 containing a conventional spin pot, now shown including a spinnerette and a spinning filter disposed between the spin pump and spinnerette. The spinnerette may be designed for the extrusion of one or more ends of filaments. Figure 1 illustrates the simultaneous extrusion of two ends 14 and 15 of multifilament, continuous filament yarn from one spinnerette. Ends 14 and 15 are extruded from the spinnerette at a rate of 15 to 34 kg (35 to 75 pounds) per hour per end, and are passed downwardly from the spinnerette into a substantially stationary column of air contained in a heated sleeve 16 of conventional height, most preferably about 38.1 cm (15 inches). The extrusion rate, of course, will differ depending on the denier and number of ends of yarn being extruded. For instance, a single continuous end of 1000 denier would be extruded from the spinnerette at a rate of about 15 to 23 kg (35 to 50 pounds) per hour, most preferably 18 kg (40 pounds) per hour, while three continuous ends would be extruded from the spinnerette at a rate of about 40 to 68 kg (90 to 150 pounds) per hour, most preferably at a rate of 55 kg (120 pounds) per hour. Yarn leaving heated sleeve 16 is passed directly into the top of the quench chamber of conventional quenching apparatus 17. The quench chamber is an elongated chimney of conventional length, preferably from 1.5 to 2.0 m (60 to 80 inches). Ends 14 and 15 of yarn are lubricated by finish applicator 18 and then the ends are separated and the filaments in each end converged by guides 19. A conventional spinning finish composition is used to lubricate the filaments. Finish applicator 18 is depicted as a lube roll which may be rotated either with or against the direction of the yarn movement; it is preferred that the lube roll rotate with the direction of yarn movement. Rotation of the lube roll is at a rate of about 1.5 to 5 revolutions per minute, typically 3.1 revolutions per minute, for a lube roll having a diameter of about 7.62 to 20.3 cm (3 to 8 inches), typically 15.2 cm (6 inches). It is preferred that the filaments be coated with from about 0.2 to about 1.0 weight percent based on the weight of the yarn of the finish, most preferably 0.5 percent. Ends 14 and 15 are then transported via interfloor tube and aspirator 20 to spin draw panel 21 (see Figure 2) where they are fed to wrap around pretension roll 23 and accompanying separator roll 23a and then feed roll 24 and accompanying separator roll 24a. From feed roll 24, the ends are then passed through conventional steam impinging draw point localizing jet 25, supplying steam at a temperature of about 460°C. to 580°C., and at a pressure of about 600 to 960 kPa absolute (75 to 125 psig), and then to a pair of draw rolls 26 and 26a. The ends pass from draw rolls 26 and 26a to relax roll 27 and accompanying separator roll 27a. The yarn ends then pass through a conventional air operated interlacing jet 28 and are taken up by winder 22.

With respect to the temperatures at which draw rolls 26 and 26a are maintained, the ultimate objective is to obtain a yarn temperature of about 190°C. to 220°C. for a given yarn residence time of about 0.25 to 0.5 second, most preferably about 0.4 second. It is believed that the best mode of achieving this objective is by maintaining both of draw rolls 26 and 26a at a temperature of 225°C to 230°C. This, however, should not be construed as discounting other acceptable draw roll temperatures such as dual rolls at a temperature of 190°C to 215°C or a single roll, preferably roll 26a, at 225°C to 230°C. In any event, it has been found that at draw roll temperatures of greater than 237°C the yarn starts sticking to the rolls, and at draw roll temperatures of less than 190°C, there is an undesirable increase in % U.E.+% T.S.

Relax roll 27 is maintained at the minimum temperature necessary to maintain temperature equilibrium during processing, preferably 60°C to 120°C.

In order to demonstrate the invention, the following Examples are given. Examples 1 to 5 and 10 are controls provided to demonstrate the effect upon yarn properties of varying the steam temperature in the localising jet 25, while Examples 6 to 9, 11 and 12 illustrate the invention. In the Examples parts and percentages are by weight unless otherwise indicated.

### Example 1

A melt of polyethylene terephthalate having an intrinsic viscosity of 0.87 to 0.96 was supplied at a rate of 17 kg (37.5 pounds) per hour per end and at a temperature of about 300°C to the apparatus shown in Figures 1 and 2. The molten polymer was fed by extruder 11 to spin pump 12 which fed spin block 13 containing a conventional spin pot as shown in Figure 1 of U.S. Patent US-A-4,072,457 to Cooksey et al. The pressure drop through the filter assembly of the spin pot averaged 200 to 400 atmospheres (20,000 to 40,000 kPa absolute). A split spinnerette designed for the simultaneous extrusion of two multi-filament ends of 192 filaments each was utilized, the spinnerette orifices having a diameter of about 0.05 cm (0.021 inch) and being spaced so that the distance between the filaments formed per end was about 0.71 to 1.0 cm (0.28 to 0.40 inch) immediately below the spinnerette.

The two ends 14 and 15 of multifilament, continuous filament yarn passed downwardly from the spinnerette into a substantially stationary column of air contained in a heated sleeve 16, about 38.1 cm (15 inches) (38.1 cm) in height, the temperature of the sleeve itself being maintained at about 400°C. Yarn leaving heated sleeve 16 was passed directly into the top of the quench chamber of quenching apparatus 17. Quenching apparatus 17 was as shown in Figure 1C of U.S. Patent US―A―3,999,910 to Pendlebury et al., hereby incorporated by reference. Quenching air at about 18.33 C. (about 65°F). and 60 percent relative humidity was supplied at about 1.9 M'/sec. (400 SCFM) to cross flow quench the filaments as they descended through the quench chamber, which had a length of about 1.7 m. (68.5 inches). The ends 14 and 15 of yarn were lubricated by finish applicator 18 and then separated and converged by guides 19. The spin finish applied consisted of 15 parts of a stearic acid ester of a mixture of secondary alcohols having the general structure where n is 5 to 6, 15 parts refined coconut oil, 13 parts of ethoxylated lauryl alcohol, 2 parts of dinonylsodium-sulfosuccinate, 5 parts ethoxylated tallow amine, 10 parts of sodium salt of alkylarylsulfonate, and 40 parts mineral oil having a boiling range between about 266°C. and 327°C. (510°F. and 620°F.). (See U.S. Patents US―A―4,103,068 and US―A―4,105,568 to Marshall et al., hereby incorporated by reference). About 0.5 weight percent of the finish composition was applied to the yarn based on the weight of the yarn. The ends were then transported via interfloor tube and aspirator 20 to the spin draw panel 21 where they were fed to wrap around a pretension roll 23 and accompanying separator roll 23a and then to feed roll 24 and accompanying separator roll 24a rotating at a speed of about 456 meters per minute. Both sets of rolls were at a temperature of less than 50°C., and the tension between pretension 23 and feed 24 rolls was about 0.03 gram per denier. From feed roll 24, the ends were then passed through conventional steam impinging draw point localizing jet 25, supplying steam at a temperature of 290°C. and at a pressure of 790 kPa absolute (100 psig.) and then to a pair of draw rolls 26 and 26a, rotating at 2,645 meters per minute. Draw roll 26a was maintained at about 130°C. to 140°C. The draw ratio was about 5.80 to 1. Yarn tension was maintained at about 0.4 gram per denier as the ends passed from draw roll 26 to relax roll 27 and accompanying separator roll 27a, the relax roll 27 being heated to 140°C. and rotating at 2,592 meters per minute. The yarn ends then passed through a conventional air operated interlacing jet 28 and were taken up by a winder 22 at a tension of from about 0.10 to 0.13 gram per denier. Table I below sets forth the physical properties and quality of the yarn so produced.

### Examples 2-8

Yarn was produced in accordance with the process of Example 1, varying only the temperature of steam in the draw point localizing jet 25 for each of Examples 2-8. Physical properties and quality of the yarn so produced are set forth in Table I.

With reference to Table I, it can be seen that increased draw point localizing jet steam temperatures resulted in reduced yarn thermal shrinkage and improved yarn dimensional stability with no adverse yarn property changes, such as lowered strength or increase elongation. This is unexpected, as a reduction in polyester yarn thermal shrinkage according to other processes normally can be achieved only by sacrificing strength or mechanical quality, by increasing the ultimate elongation or elongation at break, or by the expensive alternative of a separate operation following drawing, such as annealing.

Further, the 290°C. temperature of Example 1 was set as the lower limit for evaluation as the yarn kept breaking out and could not be strung up at draw point localizing steam temperatures below 290°C. It can be seen that % U.E.+% T.S. dropped at every draw point localizing steam temperature increase; there appears to be approximately an inverse straight line relationship such that each 10°C. rise in draw point localizing steam temperature results in about an 0.18 to 0.20 percent reduction in % U.E.+% T.S. The % T.S. is clearly reduced at each increase in draw point localizing steam temperature and shows an inverse straight line relationship with draw point localizing steam temperature between 360°C. and 520°C. where each 10°C. rise in draw point localizing steam temperature causes a 0.23 percent reduction in % T.S.

As draw point localizing steam temperature was increased, denier was slowly reduced, which indicates that less relaxing and shrinkage was occurring on the relax rolls. This would normally be expected to increase % T.S.; however, % T.S. was decreased, possibly indicating that the yarn was partially annealed at these high temperatures or the crystallinity was increased.

### Example 9

Yarn was produced in accordance with the process of Example 1 with the following variations. The melt was supplied at a temperature of about 282°C. Heated sleeve 16 was maintained at a temperature of about 300°C. Draw point localizing jet 25 was supplied with steam at a temperature of about 550°C. and at a pressure of 860 kPa absolute (110 psig). Draw roll 26a was maintained at a temperature of about 230°C., and relax roll 27 was maintained at a temperature of about 120°C. The tension between pretension 23 and feed 24 rolls was increased to 500 grams (0.08 gram per denier). Yarn tension was increased to about 1.0 gram per denier as the ends passed to relax roll 27, and winder 22 tension was increased to about 0.2 gram per denier. The draw ratio was approximately 5.9. Table II below sets forth the physical properties and quality of the yarn so produced.

With reference to Examples 8 and 9, it can be seen that whereas increased draw point localizing steam temperatures reduces % U.E.+% T.S. primarily through a % T.S. reduction, the other parameters (variations of Example 9) reduce % U.E.+% T.S. principally by reducing % U.E.

### Example 10

Yarn was produced in accordance with the process of Example 1 with the following variations. The melt had an intrinsic viscosity of about 0.68 to 0.78 and was supplied at a temperature of about 283°C. Draw point localizing jet 25 supplied steam at a temperature of about 425°C. to 430°C. Table III below sets forth the physical properties of yarn so produced.

### Example 11

Yarn was produced in accordance with the process of Example 1 with the following variations. The melt had an intrinsic viscosity of about 0.68 to 0.78 and was supplied at a temperature of about 275°C. Heated sleeve 16 was maintained at a temperature of about 250°C. Draw point localizing jet 25 was supplied with steam at a temperature of about 550°C. and at a pressure of 860 kPa, absolute (110 psig). The draw ratio was 6.2 to 1. Draw roll 26a was maintained at a temperature of about 225°C. to 230°C. Relax roll 27 was maintained at a temperature of about 115°C. while yarn tension to relax roll 27 was maintained at about 0.9 to 1.0 gram per denier. Yarn ends were taken up by winder 22 at a tension of from about 0.06 to 0.6 gram per denier, typically 0.2 gram per denier. Table III below sets forth the physical properties of the yarn so produced.

### Example 12

Yarn was produced in accordance with the process of Example 11, except that the temperature of steam in the draw point localizing jet 25 was 580°C. Physical properties of the yarn so produced are set forth in Table III below.

Note, in order to optimize process performance and product quality, the draw point localizing jet steam pressure was reduced to 790 kPa absolute (100 psig) at 580°C. Above 580°C., yarn quality and process performance were unacceptable.

A high strength dimensionally stable product is produced according to Example 11. A major advantage of this process is the ability to produce such a product from lower intrinsic viscosity polymer which is cheaper to produce as it requires less energy than high intrinsic viscosity polymer, gives increased capacity from the same equipment, and results in lower COOH, desirable for improved thermal stability.

## Claims

1. A process for the simultaneous spin-drawing of one or more ends of multifilament, continuous filament, synthetic polyester industrial fiber, comprising the steps of:
(a) supplying a melt of polyester polymer to a spinning unit;
(b) extruding the melt through a spinnerette having a plurality of extrusion orifices to form filaments;
(c) advancing the filaments through a quenching zone;
(d) lubricating the filaments;
(e) passing the lubricated filaments over a forwarding roll system maintained at a temperature of less than 50°C;
(f) subsequently passing the filaments through a steam impinging draw point localizing jet to heat the filaments substantially immediately above their second order transition temperature;
(g) passing the filaments over a pair of draw rolls;
(h) passing the filaments over a relax roll system; and
(i) winding up the filaments, characterised by, in combination;
(1) advancing the extruded filaments from step (b) through a substantially stationary column of air contained in a heated sleeve having a temperature of above 200° to 450°C before advancing the filaments through a quenching zone in step (c);
(2) employing steam at a tempeature of 482° to 580°C in the localising jet in step (f);
(3) maintaining at least one of the draw rolls at a temperature of between 190° and 237°C in step (g);
(4) maintaining the relax roll system at a temperature of 60° to 135°C and the yarn tension at 0.4 to 2.0 grams per denier in step (h); and
(5) winding up the filaments at a tension of 0.06 to 0.6 gram per denier in step (i).

2. A process according to claim 1 wherein the melt of polyester polymer is supplied at a rate of 15 to 34 kg (35 to 75 pounds) per hour per end and at a temperature of 272° to 310°C.

3. A process according to claim 1 or 2 wherein the melt of polyester polymer has an intrinsic viscosity of 0.68 to 0.96.

4. A process according to claim 1, 2 or 3 wherein during (1), the step of advancing the extruded filaments through a substantially stationary column of air, the heated sleeve has a temperature of about 250°C.

5. A process according to any one of the preceding claims wherein the steam in step (f) is at a temperature of 510° to 580°C.

6. A process according to claim 5 wherein the steam is at a temperature of about 550°C.

7. A process according to any one of the preceding claims wherein the polyester is polyethylene terephthalate.

8. A process according to any one of the preceding claims wherein during step (g) both draw rolls are maintained at a temperature of from 190° to 237°C.

9. A process according to claim 8 wherein both draw rolls are maintained at a temperature of 190° to 230°C.

10. A process according to any one of claims 1 to 7 wherein during step (g) one of the draw rolls is maintained at a temperature of 225° to 230°C. and the other draw roll is not heated.

## Patentansprüche

1. Verfahren zum gleichzeitigen Spinnstrecken eines oder mehrerer mehrfädiger kontinuierlicher Fäden aus synthetischen Polyesterindustriefasern mit den Stufen, bei denen man
a) eine Schmelze von Polyesterpolymer einer Spinneinrichtung zuführt,
b) die Schmelze durch eine Spinndüse mit mehreren Extrudieröffnungen unter Bildung von Fäden extrudiert,
c) die Fäden durch eine Abschreckzone vorrückt,
d) die Fäden schmiert,
e) die geschmierten Fäden über ein auf einer Temperatur von weniger als 50°C gehaltenes Förderrollensystem führt,
f) anschließend die Fäden durch einen durch Auftreffen von Wasserdampf einen Streckpunkt lokalisierenden Dünsenstrahl führt, um die Fäden im wesentlichen unmittelbar auf oberhalb ihrer Übergangstemperatur zweiter Ordnung zu erhitzen,
g) die Fäden über ein Paar von Streckrollen führt,
h) die Fäden über ein Entspannungsrollensystem führt, und
i) die Fäden aufwickelt, dadurch gekennzeichnet, daß man in Kombination miteinander:
(1) die extrudierten Fäden von der Stufe (b) durch eine im wesentlichen stationäre Luftsäule, die in einem erhitzten Rohr mit einer Temperatur oberhalb 200° bis 450°C enthalten ist, vorrückt, bevor man die Fäden durch eine Abschreckzone in der Stufe (c) führt,
(2) Wasserdampf mit einer Temperatur von 482° bis 580°C in dem lokalisierenden Düsenstrahl in der Stufe (f) verwendet,
(3) wenigstens eine der Streckrollen auf einer Temperatur zwischen 190° und 237°C in der Stufe (g) hält,
(4) das Entspannungsrollensystem auf einer Temperatur von 60° bis 135°C und die Garnspannung bei 0,4 bis 2,0 g je Denier in der Stufe (h) hält und
(5) die Fäden mit einer Spannung von 0,06 bis 0,6 g je Denier in der Stufe (i) aufwickelt.

2. Verfahren nach Anspruch 1, bei dem die Schmelze des Polyesterpolymers mit einer Geschwindigkeit von 15 bis 34 kg (35 bis 75 pound) je Stunde gehalten und mit einer Temperatur von 272° bis 310°C zugeführt wird.

3. Verfahren nach Anspruch 1 oder 2, bei dem die Polyesterpolymerschmelze eine grundmolare Viskositätszahl von 0,68 bis 0,96 besitzt.

4. Verfahren nach Anspruch 1, 2 oder 3, bei dem während (1), der Stufe des Vorrückens der extrudierten Fäden durch eine im wesentlichen stationäre Luftsäule, das erhitzte Rohr eine Temperatur von etwa 250°C hat.

5. Verfahren nach einem der vorausgehenden Ansprüche, bei dem sich der Wasserdampf in der Stufe (f) auf einer Temperatur von 510° bis 580°C befindet.

6. Verfahren nach Anspruch 5, bei dem sich der Wasserdampf auf einer Temperatur von etwa 550°C befindet.

7. Verfahren nach einem der vorausgehenden Ansprüche, bei dem der Polyester Polyethylenterephthalat ist.

8. Verfahren nach einem der vorausgehenden Ansprüche, bei dem während der Stufe (g) beide Streckrollen auf einer Temperatur von 190° bis 237°C gehalten werden.

9. Verfahren nach Anspruch 8, bei dem beide Streckrollen auf einer Temperatur von 190° bis 230°C gehalten werden.

10. Verfahren nach einem der Ansprüche 1 bis 7, bei dem während der Stufe (g) eine der Streckrollen auf einer Temperatur von 225° bis 230°C gehalten wird und die andere Streckrolle nicht erhitzt wird.

## Revendications

1. Procédé pour réaliser simultanément le filage-étirage d'une ou plusieurs extrémités de fibre industrielle de polyester synthétique multifilament ou à filament continu comprenant les étapes suivantes:
(a) fournir à l'état fondu un polymère de polyester à un groupe de filage;
(b) extruder le polyester fondu à travers un dispositif de filage comportant plusieurs orifices d'extrusion pour former des filaments;
(c) faire avancer les filaments à travers une zone de refroidissement brusque;
(d) lubrifier les filaments;
(e) faire passer les filaments lubrifiés sur un système d'avancement à rouleaux maintenu à une température inférieure à 50°C;
(f) faire passer ensuite les filaments à travers un jet de vapeur de localisation frappant ces derniers au point d'étirage pour chauffer les filaments sensiblement immédiatement au-dessus de leur température de transition du second ordre;
(g) faire passer les filaments sur une paire de rouleaux d'étirage;
(h) faire passer les filaments sur un système de rouleaux de détente; et
(i) embobiner les filaments, caractérisés par les étapes prises en combinaison, consistant à:
(1) faire avancer les filaments extrudés résultant de l'étape (b) à travers une colonne d'air sensiblement stationnaire contenue dans un fourreau chauffé ayant une température supérieure à 200° à 450°C avant de faire avancer les filaments à travers la zone de refroidissement brusque de l'étape (c);
(2) utiliser de la vapeur à une température de 482° à 580°C pour le jet de localisation de l'étape (f);
(3) maintenir au moins un des rouleaux d'étirage à une température comprise entre 190° et 237°C dans l'étape (g);
(4) maintenir le système de rouleaux de détente à une température de 60° à 135°C et la tension de fil à 0,4 à 2,0 grammes par denier dans l'étape (h) et
(5) embobiner les filaments à une tension de 0,06 à 0,6 grammes par denier dans l'étape (i).

2. Procédé selon la revendication 1 dans lequel le polymère de polyester à l'état fondu est fourni à un taux de 15 à 34 kg (35 à 75 Ibs) per heure par extrémité et à une température de 272° à 310°C.

3. Procédé selon l'une des revendications 1 ou 2 dans lequel le polymère de polyester à l'état fondu a une viscosité intrinséque de 0,68 à 0,96.

4. Procédé selon l'une des revendications 1, 2 ou 3 dans lequel pendant l'étape (1) consistant à avancer les filaments extrudés à travers une colonne d'air sensiblement stationnaire, le fourreau chauffé a une température d'environ 250°C.

5. Procédé selon l'une quelconque des revendications précédentes dans lequel, au cours de l'étape (f), la vapeur est à une température de 510° à 580°C.

6. Procédé selon la revendication 5 dans lequel la vapeur est à une température d'environ 550°C.

7. Procédé selon l'une quelconque des revendications précédentes dans lequel le polyester est du (poly) téréphtalate d'éthylène.

8. Procédé selon l'une quelconque des revendications précédentes dans lequel, au cours de l'étape (g) les deux rouleaux d'étirage sont maintenus à une température de 190° à 237°C.

9. Procédé selon la revendication 8 dans lequel les deux rouleaux d'étirage sont maintenus à une température de 190° à 230°C.

10. Procédé selon l'une quelconque des revendications 1 à 7 dans lequel lors de l'étape (g) un des rouleaux d'étirage est maintenu à une température de 225° à 230°C et l'autre rouleau d'étirage n'est pas chauffé.
